

## 1

3,362,910

**INHIBITED ANTIFREEZE COMPOSITION**  
 Hermann Emil Ferdinand Ordelt, Dieter Rudolf Gustav Wagnitz, and Wolfram Rudolf Walter Sokolowski, Hamburg, Germany, assignors to The British Petroleum Company Limited, London, England, a corporation of Great Britain  
 No Drawing. Filed Feb. 15, 1965, Ser. No. 432,854  
 Claims priority, application Germany, Feb. 22, 1964,  
 B 75,552  
 7 Claims. (Cl. 252—75)

**ABSTRACT OF THE DISCLOSURE**

A corrosion inhibited alcohol/water antifreeze contains mercaptothiazoline together with an alkali metal salt of tetraboric acid and alkali metal carbonate or hydroxide in the molecular ratio of 1:2-4. The composition also contains an alkali metal silicate.

This invention relates to an inhibited antifreeze composition which is particularly suitable for addition to the cooling water in motor car radiators.

Radiators of motor vehicles must be filled in winter with liquids which are not subject to the formation of ice crystals at temperatures below 0° C. Various alcohols may be mixed with the radiator water for this purpose but the most commonly used are glycerol and, particularly, ethylene glycol. A variety of materials are also incorporated for the purpose of reducing corrosive tendencies of the final composition. These additives are often mixed with the antifreeze component and the resulting mixture is usually known as an "inhibited antifreeze."

In order to obtain and advantageous power/weight relationship it is becoming common to use light metals as well as iron and non-ferrous metals in the construction of engines. In addition the engines are being operated under more and more rigorous conditions (e.g. high compression, high r.p.m. and the use of super-chargers) with the result that the operating temperature of the engine increases so that the radiator liquid has to carry away more heat. This naturally produces higher water temperatures and therefore the corrosive tendency increases.

In spite of the more stringent operating conditions it is becoming common to leave the antifreeze in the radiator for two years during both summer and winter so that servicing is reduced to topping up to replace the water which has evaporated. Thus there is an even greater need to reduce the corrosive tendencies of the radiator fluid.

As has been indicated above the radiator system of an engine often contains a variety of different metals and it is clearly important that there shall be a low corrosive tendency in respect of all the metals present in the radiator system. It is important to realise that low corrosion rates may be even more important in the case of metals which form only a small proportion of the radiator system than in the case of metals which form the bulk of the construction. Thus, for example, solder, aluminium and bearing metals have to perform an important function and relatively small amounts of corrosion on these materials may be of greater significance than much greater corrosion in respect of the main metal of construction, e.g. cast iron or steel. Thus it is an object of the present invention to reduce the corrosive tendency of antifreezes in respect of many metals which are likely to be found in a radiator system.

According to the invention an inhibited antifreeze, suitable for use in water-based radiator liquids, consists of:

- a water-miscible alcohol, preferably ethylene glycol,

## 2

- an alkali metal silicate, preferably sodium metasilicate,
- mercaptothiazoline and/or mercaptobenzothiazole,
- an alkali metal salt of tetraboric acid, preferably sodium tetraborate, and
- an alkaline reacting compound of an alkali metal, preferably sodium carbonate, sodium hydroxide, potassium carbonate or potassium hydroxide,
- at least sufficient water to maintain the other components in solution,

the molecular ratio of component (d) to component (e) being 1:2-4.

When component (e) is sodium carbonate the preferred molecular ratio is 1:3-3.5 and when component (e) is sodium hydroxide the preferred molecular ratio is 1:2.0-3.0. In addition to the ingredients just specified benzamide and/or phthalimide may be incorporated as additional ingredients.

20 A particularly suitable inhibited antifreeze composition according to the invention consists of:

|                                                    | Percent by weight |
|----------------------------------------------------|-------------------|
| Sodium metasilicate                                | 0.005-0.25        |
| 25 Mercaptothiazoline and/or mercaptobenzothiazole | 0.005-0.25        |
| Sodium tetraborate                                 | 0.26-2.6          |
| Sodium carbonate                                   | 0.28-5.6          |
| Benzamide and/or phthalimide                       | 0-0.5             |
| 30 Water                                           | 1.5-30            |
| Ethylene glycol to make 100%.                      |                   |

the molecular ratio of sodium tetraborate to sodium carbonate being 1:3-3.5.

In this example, and throughout the specification, the compositions will be given in terms of anhydrous ingredients. It will, however, usually be more convenient to prepare the compositions using hydrated materials. Thus the composition specified above would normally be prepared from borax ( $Na_2B_4O_7 \cdot 10H_2O$ ) and using this material in conjunction with anhydrous reagents the following would have to be mixed together:

|                                                    | Percent by weight |
|----------------------------------------------------|-------------------|
| Sodium metasilicate                                | 0.005-0.25        |
| 45 Mercaptothiazoline and/or mercaptobenzothiazole | 0.005-0.25        |
| Borax                                              | 0.5-5.0           |
| Sodium carbonate                                   | 0.28-5.6          |
| Benzamide and/or phthalimide                       | 0-0.5             |
| 50 Water                                           | 1.2-28            |
| Ethylene glycol                                    | to make 100%      |

The same molecular ratio of borax to sodium carbonate applies as in the previous case since there is one molecule of anhydrous sodium borate "contained" in one molecule of borax. In both cases the quantity of water should be sufficient to maintain the components in solution; in effect this means that the quantity of water is controlled by the quantity of sodium carbonate.

60 Six compositions according to the invention will now be described by way of example; these are identified as compositions I-VI. These compositions according to the invention will be compared with four other compositions illustrating borate-carbonate ratios outside the range of our invention; these comparative compositions are hereinafter identified as C1-4. The specification also includes information on prior art compositions and these are designated as P1-9.

70 The formulation of the compositions according to the invention and also of comparative compositions C1-4 are given in Table 1. In this table the figures represent

the percent by weight of the various components and the figures in the row labelled "Ratio" gives the number of molecular proportions of sodium carbonate for each molecular proportion of sodium tetraborate.

(in accordance with British specification DTD 779).

Composition P7:

|                   |       |
|-------------------|-------|
| Percent by weight | 97.5  |
| Ethylene glycol   | ----- |
| Borax             | 2.5   |

TABLE 1

| Composition                  | Invention |       |       |       |       |       | Higher and Lower Ratios |       |       |       |
|------------------------------|-----------|-------|-------|-------|-------|-------|-------------------------|-------|-------|-------|
|                              | I         | II    | III   | IV    | V     | VI    | C1                      | C2    | C3    | C4    |
| Sodium Metasilicate.....     | 0.05      | 0.05  | 0.05  | 0.05  | 0.05  | 0.05  | 0.05                    | 0.05  | 0.05  | 0.05  |
| Mercaptobenzothiazoline..... | 0.05      | 0.05  | 0.05  | 0.05  | 0.05  | 0.05  | 0.05                    | 0.05  | 0.05  | 0.05  |
| Mercaptobenzothiazole.....   |           |       |       |       |       |       |                         |       |       |       |
| Sodium Tetraborate.....      | 0.40      | 0.40  | 0.40  | 0.40  | 0.40  | 0.40  | 1.53                    | 0.26  | 1.58  | 0.26  |
| Sodium Carbonate.....        | 0.71      | 0.71  | 0.71  | 0.71  | 0.71  | 0.71  | 0.11                    | 0.10  | 0.11  | 1.10  |
| Benzoamide.....              | 0.25      |       |       |       | 0.05  |       |                         |       |       |       |
| Phthalimide.....             |           | 0.25  |       |       | 0.05  |       |                         |       |       |       |
| Ethylene Glycol.....         | 95.14     | 94.89 | 94.87 | 95.14 | 95.09 | 95.09 | 96.29                   | 93.30 | 96.29 | 93.30 |
| Water.....                   | 3.65      | 3.65  | 3.65  | 3.65  | 3.65  | 3.65  | 1.92                    | 5.24  | 1.92  | 5.24  |
| Ratio.....                   | 3.4       | 3.4   | 3.4   | 3.4   | 3.4   | 3.4   | 0.13                    | 7.9   | 0.13  | 7.9   |

(in accordance with U.S. specification OE 771a).

Composition P8:

|                   |       |
|-------------------|-------|
| Percent by weight | 95.0  |
| Ethylene glycol   | ----- |
| Sodium benzoate   | 5.0   |

Composition P9:

|                   |       |
|-------------------|-------|
| Percent by weight | 94.5  |
| Ethylene glycol   | ----- |
| Sodium benzoate   | 5.0   |

|                   |       |
|-------------------|-------|
| Percent by weight | 0.5   |
| Sodium nitrite    | ----- |

Table 2 gives the formulation of the comparative compositions designated P1-P5. As in Table 1 the figures give the percent by weight of the ingredient and the ratio gives the number of molecular proportions of sodium carbonate to each molecular proportion of borate reckoned as the total of boric acid plus sodium tetraborate plus sodium metaborate.

TABLE 2

| Composition                | P1    | P2    | P3    | P4    | P5    |
|----------------------------|-------|-------|-------|-------|-------|
| Sodium Metasilicate.....   | 0.25  | 0.31  | 0.40  | 0.15  | 0.225 |
| Mercaptobenzothiazole..... | 0.20  | 0.125 | 0.16  | 0.12  | 0.225 |
| Sodium Nitrate.....        | 0.29  | 0.365 | 0.48  | 0.18  | 0.325 |
| Sodium Nitrite.....        | 9.25  | 0.31  | 0.40  | 0.15  | 0.27  |
| Boric Acid.....            | 0.27  | 1.08  | 1.42  | 0.53  | 1.62  |
| Sodium Tetraborate.....    |       |       |       |       |       |
| Sodium Metaborate.....     | 1.0   |       |       |       |       |
| Sodium Carbonate.....      |       | 2.29  | 2.96  | 1.11  | 1.62  |
| Organic Acids.....         |       |       |       |       | 0.45  |
| Ethylene Glycol.....       | 97.74 | 95.52 | 93.98 | 97.76 | 95.49 |
| Ratio.....                 | Nil   | 1.1   | 1.2   | 0.39  | 1.9   |

The organic acids in Composition P5 were weak unsaturated acids (or their alkali metal salts) having a molecular weight of 300-350.

The remaining compositions had the following formulations:

Composition P6:

Percent by weight

|                              |      |
|------------------------------|------|
| Ethylene glycol              | 98.7 |
| Triethanolamine phosphate    | 1.0  |
| Sodium mercaptobenzothiazole | 0.3  |

For use the compositions described above are normally diluted with 1-2 parts by volume of water according to the lowest temperature expected. Tests were carried out on the corrosiveness of the various compositions to a variety of different metals and in these tests the compositions were diluted with two parts by volume of water (i.e., the test solution consisted of one-third composition and two-thirds water). The test results are given in Table 3.

TABLE 3.—CORROSION TEST ASTM 1384/61 T

| Composition | Test Metal |       |        |       |       |       |
|-------------|------------|-------|--------|-------|-------|-------|
|             | GCI        | Al    | Sn     | Cu    | Bs    | St    |
| I.....      | +0.09      | +0.12 | +0.07  | +0.04 | +0.06 | +0.07 |
| II.....     | +0.09      | +0.20 | +0.02  | +0.06 | +0.08 | +0.07 |
| III.....    | +0.09      | +0.25 | +0.04  | +0.07 | +0.08 | +0.09 |
| IV.....     | -0.10      | -0.18 | -0.12  | -0.07 | -0.11 | -0.25 |
| V.....      | -0.10      | -0.25 | -0.09  | -0.07 | -0.11 | -0.28 |
| VI.....     | -0.10      | -0.35 | -0.10  | -0.07 | -0.11 | -0.30 |
| C1.....     | -0.15      | -1.96 | -0.51  | +0.04 | -0.10 | -0.22 |
| C2.....     | -3.43      | +0.22 | -15.51 | -1.40 | -0.10 | -0.36 |
| C3.....     | -0.64      | -2.26 | -0.52  | -0.07 | -0.11 | -0.49 |
| C4.....     | -0.12      | -0.24 | -1.15  | -0.07 | -0.14 | -0.33 |
| P1.....     | +1.6       | +0.52 | +0.17  | +0.08 |       |       |
| P2.....     | +0.16      | +0.52 | +0.21  | +0.08 |       |       |
| P3.....     | +2.6       | +0    | +0.17  | +0.08 |       |       |
| P4.....     | +0.5       | +0.26 | +0.08  | +0    |       |       |
| P5.....     | +0.27      | +0.70 | +0.08  | +0.08 |       |       |
| P6.....     | +3.7       | +0.02 | +0.45  | +0.01 | +0.02 | +0.21 |
| P7.....     | +9.0       | +0.3  | +2.18  | +0.11 | +0.04 | +0.17 |
| P8.....     | +17.3      | +0.7  | +2.68  | +0.50 | +0.18 | +1.45 |
| P9.....     | +0.3       | +0.4  | +0.30  | +0.20 | +0.10 | +0.30 |

Figures indicate weight change in mg./cm.<sup>2</sup> + Indicates gain. - Indicates loss.

The column headings have the following significance:

GCI indicates grey cast iron  
 Al indicates aluminum  
 So indicates a tin/lead solder  
 Cu indicates copper  
 Bs indicates brass  
 St indicates steel

A quick inspection of Table 3 shows that only the compositions according to the invention (I-VI) and compositions P4, P5 and P9 have *all* their results less than 1.0 and therefore only these compositions will be given consideration.

The solder in the radiator system is used for making joints and a relatively small amount of corrosion of the solder may cause a leak. Thus the results in the solder column are of particular significance and it will be noted that compositions P4, P5 and P9 give results of +0.26, +0.70 and +0.30 respectively. The worst result of the compositions according to the invention was given by composition IV with a figure of -0.12. Thus there is a clear advantage in favour of our invention. Of the prior art compositions just mentioned P4 gave the best solder result but it had an aluminum result of +0.5. This figure also compares unfavourably with the worst aluminum figure according to our invention, namely -0.35. This further illustrates the superiority of the compositions according to our invention in reducing the tendency to corrosion in respect of all the metals used in the test.

Thus all the compositions according to our invention display an improvement over the comparative compositions illustrated above. It is however, interesting to note that compositions I, II and III (which contain mercaptothiazoline) gave even better results than those given by Compositions IV, V and VI (which contain mercaptobenzothiazole).

Component (c) will tend to form salts with the cation present in the antifreeze solution. If desired component (c) may be added in the form of a salt, e.g. the sodium salt.

We claim:

1. An inhibited antifreeze composition, suitable for use in water-based radiator liquids, and consisting essentially of the following ingredients:

|                                                                                                                  | Percent by weight |
|------------------------------------------------------------------------------------------------------------------|-------------------|
| (1) An alkali metal silicate                                                                                     | 0.005-0.25        |
| (2) A mercaptan selected from group consisting of mercaptothiazoline, mercaptobenzothiazole and mixtures thereof | 0.005-0.25        |
| (3) Sodium tetraborate                                                                                           | 0.26-5.0          |

Percent by weight

|    |                                                                                                                                                                                           |            |
|----|-------------------------------------------------------------------------------------------------------------------------------------------------------------------------------------------|------------|
| 5  | (4) An alkali metal compound selected from the group consisting of sodium carbonate, sodium hydroxide, potassium carbonate and potassium hydroxide                                        | 0.28-5.6   |
|    | Water                                                                                                                                                                                     | 1.5-30     |
|    | A water-miscible alcohol selected from the group of ethylene glycol and glycerol, q.s. to make 100%.                                                                                      |            |
| 10 | The molecular ratio of the sodium tetraborate to the alkali metal compound being 1:2-4.                                                                                                   |            |
| 15 | 2. A composition in accordance with claim 1 which further includes up to 0.5 % by weight of a compound selected from the group consisting of benzamide, phthalimide and mixtures thereof. |            |
|    | 3. An antifreeze according to claim 1, in which the alcohol is ethylene glycol.                                                                                                           |            |
|    | 4. An antifreeze according to claim 1 in which the silicate is sodium metasilicate.                                                                                                       |            |
| 20 | 5. An antifreeze according to claim 1, in which the alkali metal compound is sodium carbonate and the molecular ratio of component (d) to component (e) is 1:3-3.5.                       |            |
|    | 6. An antifreeze according to claim 1, in which the alkali metal compound is sodium hydroxide and the molecular ratio of component (d) to component (e) is 1:2.0-3.0.                     |            |
| 25 | 7. An inhibited antifreeze, suitable for use in water-based radiator liquids, which consists of:                                                                                          |            |
| 30 | Sodium metasilicate                                                                                                                                                                       | 0.005-0.25 |
|    | Mercaptothiazoline                                                                                                                                                                        | 0.005-0.25 |
|    | Sodium tetraborate                                                                                                                                                                        | 0.26-2.6   |
|    | Sodium carbonate                                                                                                                                                                          | 0.28-5.6   |
| 35 | A component selected from the group consisting of benzamide phthalimide                                                                                                                   | 0-0.5      |
|    | Water                                                                                                                                                                                     | 1.5-30     |
|    | Ethylene glycol to make 100%.                                                                                                                                                             |            |

the molecular ratio of sodium tetraborate to sodium carbonate being 1:3-3.5 and the quantity of water being at least sufficient to maintain the other components in solution.

References Cited  
 UNITED STATES PATENTS

45 3,015,629 1/1962 Truitt ----- 252-75  
 3,121,692 2/1964 Morehouse et al. ----- 252-75

LEON D. ROSDOL, Primary Examiner.

S. D. SCHWARTZ, Assistant Examiner.

UNITED STATES PATENT OFFICE  
CERTIFICATE OF CORRECTION

Patent No. 3,362,910

January 9, 1968

Hermann Emil Ferdinand Ordelt et al.

It is hereby certified that error appears in the above numbered patent requiring correction and that the said Letters Patent should read as corrected below.

Columns 3 and 4, TABLE 2, second column, line 4 thereof, for "9.25" read -- 3.25 --; column 5, lines 12 and 13, for "given consideration" read -- given further consideration --; line 34, for "gave" read -- give --; lines 47 and 48, for "consisting" read -- consisting of --; column 6, line 7, for "group of" read -- group consisting of --; line 24, for "claim 1, which" read -- claim 1, in which --; same column 6, after line 28, as a right-hand heading insert -- Percent by weight --.

Signed and sealed this 1st day of April 1969.

(SEAL)

Attest:

Edward M. Fletcher, Jr.

Attesting Officer

EDWARD J. BRENNER  
Commissioner of Patents